

May 15, 1951

C. G. PETERS ET AL

2,552,582

## DRY DRILLING OF DIAMONDS AND THE LIKE

Filed Dec. 23, 1946

Fig. 1



Fig. 2.

(PRIOR ART)



Fig. 3a.



Fig. 3b.



Fig. 4.



BY

INVENTORS  
CHANCEY G. PETERS  
FOREST K. HARRIS  
J. F. MOTHERHEAD  
ATTORNEY

## UNITED STATES PATENT OFFICE

2,552,582

DRY DRILLING OF DIAMONDS  
AND THE LIKE

Chauncey G. Peters, Calvert County, Md., and  
Forest K. Harris, Washington, D. C., assignors  
to the United States of America as represented  
by the Secretary of Commerce

Application December 23, 1946, Serial No. 718,093

7 Claims. (Cl. 125—30)

(Granted under the act of March 3, 1883, as  
amended April 30, 1928; 370 O. G. 757)

1

The invention herein described may be made and used by or for the Government of the United States without payment to use of any royalty therefor.

This invention relates to the drilling of diamonds and the like, and is particularly applicable in the production of wire drawing dies of such hard, crystalline material. The present invention is based on our discovery that diamonds and the like may be started and pilot drilled for the formation of the bell cones therein with greatly increased speed and with other marked advantages by impressing across a drill needle and stone condensed current and potential surges of short time duration applied to a non-rotated drill point in air or other gaseous environment with the energy of such surges controlled to maintain an energy input sufficient to produce disintegration at the point of contact by ionic bombardment but no so high as to cause a rise of temperature of the diamond that would initiate massive destruction thereof by oxidation. This discovery enables us to cause the rapid formation of a slender pilot hole or well in the diamond surface aligned with and entered by the needle point. The invention resides in the provision of a method of and apparatus for making practical application of this discovery in the drilling of diamonds.

The present invention is in part disclosed as a subcombination of the process of diamond die production forming the subject matter of our copending joint application with Walter B. Emerson, Irving L. Cooter, and Karl F. Nefflen, now Patent No. 2,438,941, issued on April 6, 1948, wherein the present invention is employed for drilling the bell in the production of diamond dies. The present invention is likewise in part disclosed in the article published within one year prior to the present application in *The American Mineralogist* 31:156-160, and entitled "Application of the High Voltage Arc to the Cutting, Sawing, and Drilling of Diamonds," by Chauncey C. Peters, one of the present applicants.

As the invention is well exemplified by the application thereof to the drilling of the bell or primary cone of a diamond die of definite size, such application is herein described as illustrative but not restrictive of the invention.

(A) *Die production in general*

In general, the production of diamond dies involves the following steps: (1) selection and preparation of die blanks, (2) spotting, or starting the hole, (3) drilling the bell or primary cone, (4)

2

drilling the secondary cone, (5) back-opening, and (6) polishing of the die surface. The present invention is particularly applicable to steps (2) and (3) of this procedure.

5

(B) *Prior art practice*

(1) (2) In accordance with the prior art, for dies of .0015 inch diameter, or less, diamonds of  $\frac{1}{16}$  to  $\frac{1}{4}$  carat, allowing a thickness of 1.3 to 1.8 millimeters, have been selected. The selected diamond has then been formed into a flat plate having two parallel surfaces spaced apart by the thickness of the die, this being generally accomplished by bruting. This blank has then been mounted and centered in a metal disc which is rotated in a bench lathe while a small conical hole is spotted or bruted in one of the flat surfaces of the stone with a diamond chip held in a pair of pliers, to act as a starting point for the drill. The blank is then ready for the drilling operation.

(3) The method and equipment developed in Europe for drilling diamond dies (see Paul Grodzinski, "Diamond and Gem Stone Industrial Production," Chap. II, page 169) essentially employ a star-drilling action. The drilling machine has a horizontal, single spindle that rotates at about 3500 revolutions per minute and carries a sewing needle for the drill. The diamond is mounted on a second spindle which oscillates the diamond against the sharpened end of the drill. Diamond dust of different grades mixed with alcohol or oil is used as the abrasive. Domestic machines as heretofore employed have operated on the same principle but usually employ ten vertical spindles to conserve space and facilitate inspection by the operator.

For drilling the primary cone, in the prior art the spotted blank is placed on the rough drilling machine, using a needle of about .040 inch diameter ground to a rather blunt point. Diamond dust of about 60 micron grade (our designation for dust having an average particle size of from 50 to 70 microns) is used for the first part of the operation, and of about 30 micron grade (25 to 35 microns) for the finish. In this way the bell is formed, preferably as a  $60^\circ$  cone of about 1 millimeter or .040 inch depth.

The time required to complete the spotting of a die by the old bruting method usually amounts to about  $\frac{1}{2}$  hour, and the time for drilling the primary cone by the old method averages from 55 10 hours to 25 hours.

(C) *Objects of the invention*

The present invention in this embodiment has for objects severally and interdependently the material reduction of the time heretofore required for starting the hole in the diamond, the provision of a new electrical dry drilling method for forming pilot wells in the diamond; and the provision of a new pilot drilling and countersinking method of forming bell cones. Further objects and advantages of the invention will be apparent from the detailed description of the illustrative embodiment of method and means incorporating its principles.

(D) *The new procedure*

Briefly, in applying the present invention in the production of small diamond dies, following preparation of the blank by any suitable method, for example, that of the copending application above mentioned, we spot drill a pilot hole in the diamond surface by our new dry drilling method, shape it to the form of a wide angle, say 90°, cone preferably by a new countersinking method employing a blunt countersinking needle and, eliminating the star drilling principle, extend a second pilot hole from the bottom of the wide angle cone by our new electrical dry drilling method, and shape the resulting funnel-shaped hole into a final primary cone which may be a 40° to 70° cone, for example, preferably by the new countersinking method.

In the accompanying drawings of embodiments illustrative of the several features of this invention:

Fig. 1 is a flow diagram of the steps of forming a primary cone in accordance with the invention.

Fig. 2 is a comparative diagram of the conventional prior art process.

Fig. 3a is a diagram of the dry drilling method and means.

Fig. 3b is a perspective view of one embodiment of dry drilling stand.

Fig. 4 is a diagram of countersinking apparatus partly in section.

Referring to Figs. 1 and 2 of the accompanying drawings, Fig. 1 illustrates diagrammatically operations performed on the blank by our new method, and Fig. 2 shows in similar diagram for reference and comparison the steps employed in the prior art. In these figures, for ease of reference the several procedural steps are numbered and described with legends showing the approximate time to perform them.

As indicated in Fig. 1, by our new procedure after the die blank has been prepared, as by cutting and polishing its facial surfaces, a pilot hole is foredrilled into the diamond by means of an electric spark, and the operation is completed by a light commercial drilling machine modified to effect countersinking. In the latter operation the rotating drill follows the pilot hole, without being deterred by axial contact with the diamond, and the conical surface of the drill, which is rotated with considerable peripheral speed, acts as a countersink or reamer for shaping the contours of the cones and applying the polish to the cone and bearing surfaces. Thus the tedious and time consuming star drilling operation, which is the basis of prior methods, is eliminated, and the strains, flaws, and fractures, and other damage to the bearing surfaces frequently resulting from preparing the blank and spotting the die by bruting, is avoided.

(1) *Preparing the blank*

In applying the present invention in the production of small diamond dies of the type disclosed in the above mentioned copending application, as the first step the blank is preferably prepared with two polished parallel surfaces and a polished window face at right angles thereto. Any desired method may be employed for preparing the blank, that disclosed in the above mentioned copending application being preferred.

For forming the bell, in accordance with the present invention the blank prepared in any suitable manner by step (1) is subjected to further steps as follows: (2) The blank is pilot drilled electrically; (3) The hole is then enlarged by mechanical countersinking; (4) The pilot hole is then extended; and (5) The bell shape may then be completed by mechanical countersinking, all as illustrated diagrammatically in Fig. 1. As there indicated, this complete operation by the present invention may be performed in from 40 to 60 minutes as compared with 10 to 25 hours by the old bruting and pecking method (Fig. 2, diagrams 2 and 3). Each of these steps will now be considered in detail.

(2) *Foredrilling the pilot hole*

For forming the pilot hole or well, step (2), Fig. 3a, apparatus is preferably used corresponding to that illustrated in Figs. 3a and 3b. As shown in Fig. 3a, the leads from the 110 volt, 60 cycle A. C. outlet are connected to the primary terminals of a zero to 120 volt output adjustable ratio autotransformer such as a variac V and the secondary of the variac is connected to the primary of a power transformer T which may be a 5000 volt, 300 volt-ampere power transformer or a 20 milliampere neon sign lighting transformer as above described. When employing the 5000 volt, 300 watt power transformer a resistance R' which may have a value of about 70 ohms is placed in the primary lead of the transformer and an A. C. ammeter A' of approximately two amperes range in the other. A capacitor C of about .001 to .008 microfarad is connected across the secondary leads of the transformer. This produces across the diamond a "condensed spark" discharge of very short duration and thus limits heating of the diamond. The rheostat R' can be dispensed with if a current limiting transformer such as a 12,000 volt, 20 milliampere neon sign lighting transformer is used instead of the power transformer.

Control and speed of drilling is improved by inserting a quenched spark gap G in the secondary lead between the transformer T and the capacitor C. This prevents the formation of a power arc follow-up in the circuit that would overheat and spoil the diamond. When this is done, however, the apparatus must be enclosed in a metallic shield S to avoid radio interference.

As shown in Fig. 3b, the drill stand for dry drilling of the pilot hole provides a metallic support for the diamond and an aligning support for the drilling needle together with electrical connections 8, 9, for connecting these two elements across the condenser C, Fig. 3a. In the simple form of stand shown in Fig. 3b for purposes of illustration, two 3-inch brass angle pieces 10, 11 are fastened to a wooden pillar 12 which is supported by the base 13. A small brass rod 14 weighing approximately 5 to 10 grams, slides closely but with minimum friction through two aligned guide holes drilled in the brass angle

pieces. Into the lower end of the rod 14 is fastened the drilling needle 15 which for the purpose of step (2) in Fig. 1 is preferably a 70% platinum, 30% iridium wire approximately .020 inch in diameter. A brass block 16 provided with an upstanding brass table 17 supports the diamond die blank 18.

With the arrangement shown in Figs. 3a and 3b it is not necessary to secure the unmounted diamond D to the pedestal 17 at all, but if desired, we contemplate effecting such securement in any suitable way, for example, by the use of a drop of cellulose acetate cement, such as that currently sold under the trade-name "Duco" cement, between the diamond and the top of the pedestal 17 to prevent shifting of the diamond relative to the electrode 18, particularly during the initial spotting operation.

In this operation the end of the drill needle 15 is ground to a cone of about 20 degrees, and the point is brought into contact with the center of the flat surface of the die blank 18. The current is then applied and adjusted by means of the variac V until a white spark extends from the needle 15 to the brass pillar 17. This should occur when the ammeter A' reads about 1 ampere. The drilling proceeds rapidly with the diamond supported in the air or other gaseous atmosphere, and is a dry drilling procedure effected without wetting of the stone or immersion of it in any electrolyte. If the end of the drill 15 becomes red the current should be reduced by adjusting the variac V until the color disappears. The current should, however, be sufficient to maintain the white spark between the drill 15 and the pillar 17. In about 20 minutes time a roughly cylindrical hole, Fig. 1, step (2), about 0.5 mm. (0.020 inch) deep and .2 mm. (0.008 inch) in diameter, is drilled in the diamond and the end of the drill 15 is disintegrated. Very little progress is made at this point by repeating the dry drilling operation with a re-sharpened needle.

### (3) Countersinking

According to our invention, therefore, the foredrilled blank 18 is next mounted on the light drilling machine employing a suitable blunt or wide-angled countersink, for example, a No. 1 drill needle, sharpened to a 90° cone and rotated at a relatively high speed, for example, 3200 R. P. M. Using grade 45 micron powder in alcohol or any other suitable vehicle, and reciprocating the diamond axially of the needle at a slow rate, say 200 times per minute, so that the powder may enter between the needle point and diamond surface, the bell cone is then countersunk to the bottom of the foredrilling as indicated in Fig. 1, step (3), in about 45 minutes. During this operation the die is applied against the countersinking point about  $\frac{1}{3}$  of the time with a very light pressure, of the order of a few grams, and the distance of reciprocation of the diamond away from the needle point may be of the order of a half millimeter.

Suitable apparatus for the performance of this step is diagrammatically illustrated in Fig. 4 in which the drill needle 20 is carried by a vertical shaft 21 rotated in a bearing 22 by any suitable means as the cord and pulley drive 23. The diamond 18 is mounted on a support 24, which is shown as provided with a height adjusting means 25, and carried by an arm 26 pivoted at 27 and adapted to raise and lower the support 24 as aforesaid. In the form shown a lightly loaded

counterweight 28 lifts the diamond against the drillpoint, and the arm reciprocating cam 29, suitably driven, effects the displacement of the blank 18 from contact with the drill point.

- 5 For convenience in the machine drilling, the blank 18 is mounted in a newly developed small window-nib illustrated in Fig. 4. This nib, in the form shown, comprises a cylindrical cup-shaped member 30 provided with two diametrically aligned viewing openings 31 and with a close fitting cylindrical plug 32 having a conical reservoir 33 to hold the dust-and-vehicle mixture. The reservoir 33, as shown, narrows to an axial center opening, and the diamond blank is sealed to the plug 32 by a thin layer of wax on the bottom of the plug in the space 34 surrounding this center opening. This layer of wax prevents leakage of the cutting mix and also enables the blank 18 to be lifted from the cup 30 by lifting out the plug 32, which may be provided with a flange around its upper end to facilitate its removal, if desired. Beeswax, dental wax, or the like, makes a good seal from which the diamond is easily disengaged. The window on the diamond, when it is secured in the nib, is aligned with the openings 31, so that the progress of the drilling may be seen through one of these openings, the blank being illuminated by light shining through the other. With this unit the blank 30 18 can be mounted or unmounted in a few moments.

### (4) Pilot extension

- In the next step, Fig. 1, step (4), by repeating the dry drilling operation of step (2) (see Figs. 3a-3b) the foredrilling is extended an additional 0.5 mm. (0.020 inch) in about 20 minutes.

### (5) Finishing the bell

- Following the pilot extension the blank is again returned to the drilling machine, and further countersunk with a needle ground to a 60° cone, as shown in Fig. 1, step (5). Using grade 20 micron powder at the start and grade 6 micron powder to finish, a smooth 60° cone about 1.0 mm. (.040 inch) deep is obtained in about an hour. The set-up is generally like that employed in step (3) (see Fig. 4). At this point about 0.2 mm. (.008 inch) of the blank thickness should be left for the secondary cone. If the finished blank is to be more than 1.2 mm. thick, say 1.6 mm., further foredrilling and countersinking of the bell may be practiced.

### (6) Further treatment

- After formation of the bell in accordance with the present invention, the secondary cone of the die may be formed in any suitable manner, and the die may then be completed by back-opening and blending and polishing as desired. Preferably these operations are performed in accordance with the method disclosed in the above mentioned copending application, but such further procedure forms no part of the present invention.

### (7) Economies

- In forming a bell cone employing the present invention, the foredrilling and countersinking, repeated until the desired depth of bell is obtained, may be effected in about 3 hours per die. One operator can care for two electric drills or ten countersinking spindles, and thus the time required for forming a bell by the present invention becomes approximately 40 to 60 man minutes per die.

By contrast, in the prior art bruting and pecking method an average of 2.5 man hours is required per bell, and in addition considerable consumption of diamond chips and powder is involved in the bruting and pecking operations.

Thus the present invention effects a noteworthy saving of material, labor, and time, aside from producing a better and more uniform bell which in its initial production is generated with a well polished surface. These and other advantages may be more fully appreciated from a consideration of the aforesaid copending application and publication, to which reference is made in this connection.

From the foregoing description of a preferred method and apparatus illustrative of the invention, it will be appreciated that the invention is not limited to the precise embodiment disclosed, but includes modifications thereof, as will be apparent from the appended claims. Reference is also made to the aforesaid publication which discloses a further embodiment of the present invention exemplifying some of the modifications which may be made without departing from the broader aspects of the invention. Thus, in lieu of the sliding mounting of the needle 14-15 in brackets 10-11 (Fig. 3b) the needle-holder 14 may be suspended from a light coil spring, and this assemblage may be lowered to rest the tip of the needle 15 against the diamond with a suitable pressure. While pressures up to 10 grams may be employed, a pressure of about 0.5 gram gives extremely good results.

The needle 15 may have diameters other than 0.020 inch, but this particular diameter is especially efficacious. During the drilling operation best results are obtained with the primary current adjusted to a value which is just below that causing a needle of 0.020 inch diameter to rise to a visible red heat. The limiting condition for rapid drilling seems to be the power that can be applied before frosting of the diamond occurs. Frosting never results when the exposed 0.020 inch diameter electrode is operated below its reddening temperature. With a 0.032 inch diameter electrode frosting occurs without visible reddening. Therefore, the 0.020 inch electrode enables the selection of the best power value for efficient drilling. With such electrode the variac V is adjusted until the 0.020 needle begins to show incandescence and the input voltage is then reduced to the point at which the redness disappears.

As the drilling nears the bottom of the diamond, current tends to be conducted through the diamond, discharge around the diamond ceases, and the diamond tends to overheat. Conductive perforation of thin webs remaining in diamonds after formation of bell and outlet cones therein by other methods forms no part of the present invention and is disclosed in the U. S. patent to Kurtz et al. No. 2,377,159, which effects the perforation of the thin web so quickly that the heating problem is not there encountered. The heating problem here referred to is incident to the prolonged drilling of pilot wells by ionic bombardment. In practicing the present invention the tendency to overheat when the drilling approaches the bottom of the diamond may be overcome by mounting the diamond being drilled upon another flat surfaced diamond silver soldered in a cavity in the block 16 and protruding about 0.5 mm. above the metal surface. The pedestal 17 is dispensed with in this arrangement.

In the practice of this invention, the elec-

trode preferably is tapered to a tip diameter of from 0.002 to 0.003 inch, and the electrode is preferably given an occasional rotation of a fraction of a turn. This procedure tends to result

- 5 in the uniform production of a well-shaped symmetrical hole. In the dry drilling of the pilot holes, it is also desirable to drill for about ten minutes and then continue the drilling with a re-sharpened electrode for another ten minutes,
- 10 in lieu of continuously employing the same electrode for a 20 minute drilling period. It is also desirable to employ protective glasses while observing the condition of the spark during the drilling operation, to avoid injury to the operator's eyes.

What is claimed is:

1. A method of dry drilling pilot wells in diamonds and like hard, crystalline stones which comprises supporting the diamond in a gaseous atmosphere on an electrically conductive base, pressing lengthwise against the diamond an electrically conductive needle point, creating a condensed electrical spark discharge around said diamond between said needle point and base,
- 20 controlling the power input of said condensed spark discharge to cause disintegration of the diamond at the needle contact area by ionic bombardment without heating the diamond to a temperature causing massive destruction thereof
- 30 by oxidation, and continuing such controlled condensed spark discharge for a time sufficient to produce a well in the diamond aligned with and entered by said needle point.

2. A method of dry drilling pilot wells in diamonds and like hard, crystalline stones which comprises supporting the diamond in a gaseous atmosphere on an electrically conductive base, pressing endwise upon the diamond—with a pressure of about 0.5 to 10 grams—the tip of a platinum-iridium wire having a diameter of about 0.02 inch, creating a condensed electrical spark discharge around said diamond between said wire and said base, controlling the power input of said condensed spark discharge to cause disintegration of the diamond on the needle contact area by ionic bombardment without heating the diamond to a temperature causing massive destruction thereof by oxidation and continuing said discharge until a well has been formed in the diamond having a depth of about 0.02 inch and a width at its top of about 0.008 inch.

3. A method of dry drilling diamonds and like hard, crystalline stones which comprises electrically foredrilling a pilot well in the diamond by the method of claim 1, and thereafter countersinking said well with a rotating blunt needle point and diamond dust to a depth approaching the depth of said pilot well.

4. A method of dry drilling diamonds and like hard, crystalline stones which comprises electrically foredrilling a pilot well in the diamond by the method of claim 1, then countersinking said well with a rotating blunt needle point and diamond dust to a depth approaching the depth of said pilot well, and then drilling by the method of claim 1 a further well extending from the bottom of the countersunk well.

5. A method of dry drilling diamonds and like hard, crystalline stones which comprises electrically foredrilling a pilot well in the diamond by the method of claim 1, then countersinking said well with a rotating blunt needle point and diamond dust to a depth approaching the depth of said pilot well, then foredrilling a second pilot well from the bottom of the countersunk well by

the method of claim 1, and thereafter further countersinking the well to a depth approaching the total depth of the second well.

6. Apparatus for dry drilling pilot wells in diamonds and like hard, crystalline stones comprising an electrically conductive base for supporting the diamond, a needle-like drill point, means for pressing said drill point endwise towards said base, and against a diamond supported thereon, a condensed spark discharge circuit connected across said needle and base, said discharge circuit comprising the secondary of a high voltage transformer, a quenched spark gap and a capacitor connected to be charged from the transformer secondary through the gap, said capacitor being connected in parallel with the path between said drill point and base, and means for adjusting the power in said condensed spark discharge circuit to a value sufficiently high to create a spark discharge around the diamond embraced between said needle and base and effect disintegration of the diamond at the needle contact area by ionic bombardment but not so high as to heat the

diamond to a temperature producing massive destruction of the diamond by oxidation, so as to produce a well in the diamond aligned with and entered by said needle point.

5 7. Apparatus according to claim 6, said drill point being formed of platinum-iridium wire having a diameter of about 0.02 inch.

CHAUNCEY G. PETERS.  
FOREST K. HARRIS,

10

#### REFERENCES CITED

The following references are of record in the file of this patent:

#### UNITED STATES PATENTS

|    | Number    | Name            | Date          |
|----|-----------|-----------------|---------------|
| 15 | 971,935   | Simon           | Oct. 4, 1910  |
|    | 1,922,497 | Peterson        | Aug. 15, 1933 |
|    | 2,258,480 | Bergmann et al. | Oct. 7, 1941  |
| 20 | 2,300,855 | Allen et al.    | Nov. 3, 1942  |
|    | 2,377,159 | Kurtz et al.    | May 29, 1945  |
|    | 2,398,250 | Robbins         | Apr. 9, 1946  |
|    | 2,452,141 | Pasdertz        | Oct. 26, 1948 |